

# UNITED STATES PATENT OFFICE.

MAX SMETANA, OF PHILADELPHIA, PENNSYLVANIA.

## ADHESIVE COMPOSITION.

No. 879,013.

Specification of Letters Patent.

Patented Feb. 11, 1908.

Application filed March 20, 1907. Serial No. 363,482.

To all whom it may concern:

Be it known that I, MAX SMETANA, subject of the Emperor of Austria-Hungary, residing at Philadelphia, in the county of Philadelphia and State of Pennsylvania, have invented certain new and useful Improvements in Adhesive Compositions, of which the following is a specification.

My invention has relation to adhesive compositions; and it contemplates the provision of an economical adhesive composition possessed of a high degree of elastic binding power and calculated to save in the production of work by expeditiously drying, and one which by reason of its nature is adapted to be deposited in sufficient quantity for strong binding on the surface of a part that is to be connected to another part and yet is not liable to penetrate to an undue extent into the material of the said part.

My composition consists of glue made according to the ordinary, well known formula or any other formula consonant with the purpose of my invention, and finely subdivided fibers, preferably fibers from paper and cellulose, though other fibers possessed of capillary characteristics and insoluble in water, such for instance as fibers from leather, linen, wool, cotton, silk, hair, wood, and analogous materials, may be employed without involving departure from the scope of my invention as defined in the claims appended.

In the preferable practice of my invention, the finely subdivided fibers are mixed with glue prepared in the usual way but not dried and not quite finished; the proportion of the fibers to the glue depending on the character of the parts to be connected. The proper proportion of fibers is best determined by applying a thin layer of glue to the surface of the part to be connected, and observing after the lapse of a short period when all of the fibers are saturated, if there is an adequate layer of fibers on the glued surface—i. e., a layer sufficient to assure the proper binding of the part to another part. This is particularly true when leather, paper and soft woods are to be glued.

The fibers mixed with the glue take up by capillary attraction the moisture of the glue and give off such moisture to the atmosphere or in other words serve as a siccative; and it will also be manifest that the fibers render the adhesive mixture tough and elastic, that

55 they assure the surfaces of the parts to be con-

nected being jagged and calculated to closely fit each other, and that by settling on the surface of the glue they contribute materially to the strong and durable cohesion of the parts. This latter is especially characteristic of my 60 composition when the same is employed in the connection of parts of wood, leather and paper.

It will be gathered from the foregoing that my composition is advantageous, because the 65 fibers, while enhancing the binding strength of the composition render the same much cheaper than a corresponding quantity of glue alone; also, that the fibers, by preventing penetration of an undue quantity of glue 70 into the material or materials of the parts connected effect a saving of glue, and this while expediting drying of the glue and composition as a whole, and in that way contributing to the cheapness of the work produced. 75

When cheap production of work is sought, I use paper fibers because of the facility and cheapness with which the same may be produced.

While I have designated glue as the preferable adhesive material my invention consists broadly in the combination of fiber substantially as specified with any suitable adhesive substance as for instance starch paste, flour paste, dextrin, albumen, shoemaker's pulp, 85 etc.

Having described my invention, what I claim and desire to secure by Letters Patent, is:—

1. An adhesive composition capable of adhering to the surface of a part that is to be connected to another part and comprising an adhesive substance, and fibrous material commingled with the adhesive substance for taking up moisture from the same and giving 95 off such moisture to the atmosphere to accelerate drying of the composition; the proportion of adhesive substance being sufficient to saturate all of the fibres of the fibrous material.

2. An adhesive composition capable of adhering to the surface of a part that is to be connected to another part and comprising an adhesive substance and a fibrous material combined therewith; the proportions of the 105 ingredients being such as to assure the provision on the adhesive substance of a layer of fibers sufficient for the proper binding of the part to another part.

3. An adhesive composition capable of ad-

100

105

110

hering to the surface of a part that is to be connected to another part and comprising glue and a fibrous material combined therewith; the proportions of the ingredients being such as to assure the provision on the glue of a layer of fibers sufficient for the proper binding of the part to another part.

4. An adhesive composition capable of adhering to the surface of a part that is to be connected to another part and comprising an adhesive substance and fibrous material commingled with the adhesive substance for taking up moisture from the same and giving off such moisture to the atmosphere to accelerate drying of the composition; the proportion of adhesive substance being sufficient to saturate all of the fibers of the fibrous material and such as to assure the provision on the adhesive substance of a layer of fibers sufficient

for the proper binding of the part to another 20 part.

5. An adhesive composition capable of adhering to the surface of the part that is to be connected to another part and comprising glue and fibrous material possessed of capillarity and insolubility, commingled with the glue; the proportion of glue being sufficient to saturate all the fibers of the fibrous material and such as to assure the provision on the glue of a layer of fibers sufficient for the 25 30 proper binding of the part to another part.

In testimony whereof I affix my signature in presence of two witnesses.

MAX SMETANA.

Witnesses:

BERNHARD T. MILLS,  
H. MEIER.